# EUROPEAN PATENT SPECIFICATION

(11) **EP 4 602 196 B1**
(45) Date of publication and mention of the grant of the patent: **13.05.2026**
(21) Application number: 23777264.5
(22) Date of filing: 26.09.2023
(51) Int. Cl.: C25B 1/23, C25B 3/03, C25B 3/07, C25B 3/26, C25B 9/19, C25B 11/032, C25B 15/08

(54) **CO2 ELECTROREDUCTION TO MULTI-CARBON PRODUCTS IN ACIDIC CONDITIONS COUPLED WITH CO2 REGENERATION FROM CARBONATE**
CO2-ELEKTROREDUKTION ZU MEHRKOHLENSTOFFPRODUKTEN IN SAUREN BEDINGUNGEN IN VERBINDUNG MIT CO2-REGENERATION AUS CARBONAT
ÉLECTRORÉDUCTION DE CO2 EN PRODUITS MULTICARBONES DANS DES CONDITIONS ACIDES COUPLÉE À UNE RÉGÉNÉRATION DE CO2 À PARTIR DE CARBONATE

(30) Priority: 13.10.2022 EP 22315237
(43) Date of publication of application: 20.08.2025
(73) Proprietor: TotalEnergies OneTech, 92400 Courbevoie (FR); College de France, 75231 Paris Cedex 05 (FR)
(72) Inventor: SCHREIBER, Moritz Wilhelm, 7181 Seneffe (BE); PERAZIO, Alessandro, 75005 Paris (FR); FONTECAVE, Marc, 75005 Paris (FR); CREISSEN, Charles E., Manchester WA15 9JA (GB)
(74) Representative: Mellet, Valérie Martine
(86) International application number: PCT/EP2023/076572
(87) International publication number: WO 2024/078866

(56) References cited:
- WO-A1-2019/051609
- US-A1- 2020 080 211
- VERMAAS DAVID A. ET AL: "Synergistic Electrochemical CO 2 Reduction and Water Oxidation with a Bipolar Membrane", ACS ENERGY LETTERS, vol. 1, no. 6, 10 November 2016 (2016-11-10), American Chemical Society, pages 1143 - 1148, XP055897569, ISSN: 2380-8195, DOI: 10.1021/acsenergylett.6b00557

## Description

### Technological field

The present disclosure relates to processes and systems comprising a gas-fed flow cell for electrochemical carbon dioxide reduction, for example, to upgrade greenhouse gases such as carbon dioxide to valuable fuels and feedstocks.

### Technological background

Electrochemical carbon dioxide reduction (CO₂R) offers a sustainable route to generate valuable chemical products from CO₂ and renewable electricity sources. Recent progress has brought CO₂R closer to commercial viability through the development of devices that overcome the severe limitations of mass transport arising from the low solubility of CO₂ in aqueous solutions. One example is the gas-fed flow cell, in which the CO₂ is supplied as a gas through the back of a gas-diffusion electrode (GDE) in contact with a flowing electrolyte solution. These devices can regularly attain high current densities (hundreds of mA cm⁻²) at low overpotentials (<1 V). However, the common use of alkaline or neutral pH electrolyte solutions has prohibited high conversion yields due to the unwanted reaction of CO₂ with hydroxide ions, which results in reactant loss through the formation of (bi)carbonate (Figure 3a).

These species can be externally converted back to CO₂, but the regeneration process accounts for more than half of the energy required for the electrolyser in the case of an alkaline flow cell.

The problem can be partly addressed by using acidic electrolyte solutions where the pH is below the pKa of bicarbonate formation. In such systems, while the CO₂ is still converted to (bi)carbonate (Eq.1 and Eq. 2) by the alkaline local pH at the cathode arising from hydroxide ions generated during CO₂ reduction (Eq. 3), these (bi)carbonate species are immediately converted back to CO₂ (termed r-CO₂ as this is regenerated) due to the low bulk pH (Eq. 4). (Figure 3b). This provides the possibility to recycle and re-react the r-CO₂, which maximizes the conversion yield of the CO₂R since all the reactant is ultimately converted into reduction products and is not permanently lost as (bi)carbonate.

CO₂ + OH⁻ HCO₃⁻ Equation 1

HCO₃⁻ + OH⁻ CO₃²⁻ + H₂O Equation 2

CO₂ + H₂O + 2e⁻ CO + 2 OH⁻ Equation 3

HCO₃⁻ + H⁺ r-CO₂+ H₂O Equation 4

However, a major fraction of input CO₂ is consumed by the electrolyte through reactions with the hydroxide to form carbonate/bicarbonate in both alkaline and neutral reactors. Acidic routes for CO₂R have been studied to overcome this limitation. However, it was found that the acidic route also promotes the hydrogen evolution reaction (HER).

X. Huang et al., in Science, 2021, 372, 1074-1078 report that concentrating potassium cations in the vicinity of electrochemically active sites accelerates CO₂ activation to enable efficient CO₂R in acid. CO₂R was achieved on copper at pH <1 with a single-pass CO₂ utilization of 77%, including a conversion efficiency of 50% toward multicarbon products (ethylene, ethanol, and 1-propanol) at a current density of 1.2 amperes per square centimeter and a full-cell voltage of 4.2 volts.

Y. Xie et al., in Nature Catalysis, 2022, 5, 564-570, report a design strategy that suppresses hydrogen evolution reaction activity by maximizing the co-adsorption of CO and CO₂ on Cu-based catalysts to weaken H* binding. Using density functional theory studies, it was found Pd-Cu promising for selective C₂₊ production over C₁, with the lowest ΔG_{OCCOH*} and ΔG_{OCCOH*} - ΔG_{CHO*}. Pd-Cu catalysts were synthesized and reported a crossover-free system (liquid product crossover <0.05%) with a Faradaic efficiency of 89 ± 4% for CO₂ to C₂₊ at 500 mA cm⁻², simultaneous with single-pass CO₂ utilization of 60 ± 2% to C₂₊.

J. Gu et al., in Nature Catalysis, 2022, 5, 268-276, show that by suppressing the otherwise predominant hydrogen evolution using alkali cations, efficient CO₂ electroreduction can be conducted in an acidic medium, overcoming the carbonate problem. The cation effects are general for three typical catalysts including carbon-supported tin oxide, gold, and copper, leading to Faradaic efficiency of as high as 90% for formic acid and CO formation. The analysis suggests hydrated alkali cations physisorbed on the cathode modify the distribution of electric field in the double layer, which impedes hydrogen evolution by suppressing the migration of hydronium ions while at the same time promoting CO₂ reduction by stabilizing key intermediates.

Although the above techniques are promising, there is still room for improvement. For example, the use of proton exchange membranes leads to a crossover of metal ions, cationic electrolyte species, and products, which can negatively impact device performance and stability over long durations. The use of acidic anolytes requires acid-tolerant oxygen evolution reaction (OER) catalysts based on precious metals such as Ir or Ru, which increase the costs involved.

WO2019/051609 discloses processes and apparatus for electrocatalytically reducing carbon dioxide are described. The process may include: providing a gas containing carbon dioxide at a cathode of an electrolytic cell comprising a membrane electrode assembly which includes a bipolar membrane separating an anode from the cathode. A support layer containing water is located between the bipolar membrane and the cathode. An electrical potential difference between the cathode and the anode of the membrane electrode assembly electrocatalytically reduces the carbon dioxide to carbon monoxide or another useful chemical. The support layer facilitates stable operating at higher current densities.

US2020/080211 discloses an electrolysis cell comprising: a cathode space housing a cathode; a first ion exchange membrane including an anion exchanger and adjoining the cathode space; an anode space housing an anode; a second ion exchange membrane including a cation exchanger and adjoining the anode space; and a salt bridge space disposed between the first ion exchange membrane and the second ion exchange membrane. The cathode comprises: a gas diffusion electrode having a porous bound catalyst structure of a particulate catalyst on a support; a coating of a particulate catalyst on the first and/or second ion exchange membrane; and a porous conductive support impregnated with a catalyst.

Vermaas David et al. « Synergistic Electrochemical CO2 reduction and Water Oxidation with Bipolar Membrane" (DOI: 10.1021/acsenergylett.6b00557) reads that the electrochemical conversion of CO₂ and water to value-added products still suffers from low efficiency, high costs, and high sensitivity to electrolyte, pH, and contaminants. Here, we present a strategy for this reaction using a silver catalyst for CO₂ reduction in a neutral catholyte, separated by a bipolar membrane from a nickel iron hydroxide oxygen evolution catalyst in a basic anolyte. This combination of electrolytes provides a favorable environment for both catalysts and shows the effective use of bicarbonate and KOH to obtain low cell voltages. This architecture brings down the total cell voltage by more than 1 V compared to that with conventional use of a Pt counter electrode and monopolar membranes, and at the same time, it reduces contamination and improves stability at the cathode.

There is still a need for improvement of processes and systems for efficient electrochemical carbon dioxide reduction (CO₂R) reactions.

### Summary of the disclosure

One or more of the above needs can be fulfilled by the process and system according to the present disclosure wherein the system comprises a gas-fed flow cell with a bipolar membrane and an acidic catholyte flow comprising one or more alkali metal cations.

According to a **first aspect,** the disclosure provides **a process** for electrolysing carbon dioxide, said process is remarkable in that it comprises the following steps:
a) providing a system comprising a gas-fed flow cell comprising a gas chamber with a gas inlet, a gas outlet, a catholyte chamber, and a gas diffusion electrode comprising a metal-based catalyst, wherein the gas diffusion electrode is placed between the gas chamber and the catholyte chamber;
b) providing a catholyte flow and an anolyte flow into said gas-fed flow cell;
c) activating said gas diffusion electrode under operating conditions;
d) providing a gas input flow comprising carbon dioxide using the gas inlet of the gas chamber to produce a direct gas stream exiting from the gas outlet of the gas chamber and a liquid catholyte output flow from the catholyte chamber comprising products, wherein said liquid catholyte output flow is degassed in a catholyte reservoir to produce an indirect gas stream exiting from a gas outlet of the catholyte chamber;
wherein the catholyte flow is an acidic catholyte flow comprising one or more alkali metal cations and in that the gas-fed flow cell comprises a bipolar membrane includes a cation-exchange layer (CEL) in contact with the catholyte and an anion-exchange layer (AEL) in contact with the anolyte; wherein the cation-exchange layer provides protons to the catholyte and the anion exchange layer provides hydroxide ions to the anolyte; in that the acidic catholyte has a pH of at most 5.5 and in that the catholyte pH is less than the anolyte pH.

With preference, the indirect gas stream exiting from the catholyte reservoir comprises carbon dioxide, and the process further comprises a step e) of recovering the indirect gas stream exiting from the catholyte reservoir and recycling said indirect gas stream into the gas input flow comprising carbon dioxide of step d).

With preference, the indirect gas stream exiting from the catholyte reservoir comprises at least 90 mol.% of CO₂ based on the total molar content of the indirect gas stream; preferably at least 95 mol.%; more preferably at least 98 mol.%.

Surprisingly, it has been found that it was possible to operate a system comprising a gas-fed flow cell in a way that enhances carbon dioxide regeneration from generated carbonate in the catholyte. The process of the disclosure not only provides good single-pass conversion to CO₂R products (SPC) but also favours the recovery of the carbon dioxide that was converted into (bi)carbonate to recycle it back to the cell, to have it react again with the catalyst. This results in the CO₂R product conversion yield being increased and avoids the loss of CO₂. Existing devices and processes for acidic CO₂R have relied on proton exchange membranes (PEMs), such as Nafion^{®}, to separate the anode and the cathode compartments (Figure 3c). However, PEMs cannot maintain a pH gradient, the anolyte has to be acidic. The use of a bipolar membrane in the process and system of the disclosure allows, among other advantages, an asymmetric setup wherein acidic CO₂R is performed using an alkaline anolyte.

According to a **second aspect,** the disclosure provides a system suitable to perform the process of electrolysing carbon dioxide according to the first aspect, the system comprises a gas-fed flow cell comprising a gas chamber, a catholyte chamber, and an anolyte chamber, wherein said gas chamber is separated from the catholyte chamber by a gas diffusion electrode, said gas diffusion electrode having a gas diffusion membrane being comprised within said gas chamber, wherein said catholyte chamber and said anolyte chamber comprise respectively a cathode and an anode, and wherein the system further comprises catholyte and anolyte and means to flow the catholyte and the anolyte within respectively said catholyte chamber and said anolyte chamber;
wherein the system is remarkable in that the catholyte flow is an acidic catholyte flow comprising one or more alkali metal cations, in that the gas-fed flow cell comprises a bipolar membrane includes a cation-exchange layer in contact with the catholyte and an anion-exchange layer in contact with the anolyte; wherein the cation-exchange layer provides protons to the catholyte and the anion exchange layer provides hydroxide ions to the anolyte; in that the acidic catholyte has a pH of at most 5.5 and in that the catholyte pH is less than the anolyte pH; wherein, the system further comprises a catholyte reservoir configured to receive and degas the output flow exiting the catholyte chamber, and with preference means to recover an indirect gas stream exiting the gas outlet of the catholyte reservoir and means to recycle the said indirect gas stream back into the gas chamber.

One or more of the following features advantageously further define the process and/or the system of the disclosure.

For example, the gas input flow provided in step (d) has a flow rate ranging from 0.5 to 10 mL/min; preferably from 0.6 to 5 mL/min; more preferably from 0.7 to 3.5 mL/min; even more preferably from 0.8 to 3.0 mL/Min; most preferably from 0.9 to 2.8 mL/min; and even most preferably from 1.0 to 2.5 mL/min or from 1.1 to 1.8 mL/min. It is understood that the above values are given for a cell wherein the dimensions are 7.5cm x 7.5 cm x 3.2 cm. These values will be adapted by the person skilled in the art without difficulties in case the dimensions of the cell are changed.

For example, the acidic catholyte has a pH ranging from 0.5 to less than 5.5; preferably from 0.5 to 5.4 or from 0.6 to 5.4; more preferably from 0.7 to 5.2; even more preferably from 0.8 to 5.4 or from 0.8 to 5.0; most preferably from 0.9 to 4.5; even most preferably from 1.0 to 4.0 or from 1.1 to 3.5.

For example, step b) comprises providing a catholyte flow and an anolyte flow wherein the catholyte pH is less than the anolyte pH.

For example, the anolyte has a pH ranging from 7 to 15; preferably from 10 to 14, allowing non-noble metal catalysts (OER catalyst, stainless steel, Ni foam).

For example, the acidic catholyte comprises one or more acids at a concentration ranging from 0.001 to 5.0 M; preferably from 0.005 to 3.0 M or from 0.01 to 2.0 M; or from 0.05 to 1.5 M or from 0.01 to 1.0 M.

For example, the acidic catholyte comprises one or more acids at a concentration ranging from 0.01 to 1.0 M and one or more alkali metal cation donors at a concentration ranging from 0.5 to 5.0 M. With preference, the one or more alkali metal cations are weakly hydrated cations and/or the one or more alkali metal cations are one or more selected from Cs⁺, K⁺, Li⁺ and Na⁺; preferably the one or more alkali metal cations are or comprise K⁺.

For example, the acidic catholyte comprises one or more alkali metal cation donors selected from caesium chloride, caesium iodide, caesium sulfate, caesium phosphate, caesium hydroxide, potassium chloride, potassium phosphate monobasic, potassium sulfate, potassium iodide, potassium hydroxide, lithium chloride, lithium iodide, lithium sulfate, lithium phosphate, lithium hydroxide, sodium chloride, sodium sulphate, sodium iodide, sodium phosphate, and sodium hydroxide; preferably selected from potassium chloride, potassium phosphate monobasic, potassium sulfate, potassium iodide, and potassium hydroxide; more preferably the one or more alkali metal cation donors are or comprise potassium chloride.

With preference, the one or more alkali metal cation donors at a concentration ranging from 0.5 to 5.0 M; preferably ranging from 1.0 to 4.5 M; and more preferably ranging from 2.0 to 4.0 M.

For example, the acidic catholyte comprises one or more acids selected from hydrochloric acid, sulfuric acid, hydrobromic acid, hydriodic acid, perchloric acid, and chloric acid; preferably sulfuric acid. With preference, the one or more acids are present at a concentration ranging from 0.01 to 1.0 M; preferably, from 0.02 to 0.5 M; more preferably ranging from 0.03 to 0.2 M.

In an embodiment, step (a) of providing a system comprising a gas-fed flow cell comprises preparing said gas-fed flow cell by spray-coating an ink comprising an ion-conducting polymer and a metal-based catalyst on a gas diffusion membrane. Therefore, the gas-fed flow cell comprises a spray-coated ink on a gas diffusion membrane, wherein the ink comprises an ion-conducting polymer and a metal-based catalyst.

In an embodiment, the metal-based catalyst is provided in the form of nanoparticles having an average diameter ranging from 5 nm to 200 nm as measured by transmission electron microscopy, preferably from 10 nm to 150 nm, more preferably from 20 nm to 100 nm.

For example, the metal of the metal-based catalyst is selected from copper, silver, and any mixture thereof; with preference, the metal-based catalyst is or comprises copper oxide nanoparticles.

For example, the metal-based catalyst is or comprises copper oxide nanoparticles and the process comprises a catalyst activation step to reduce copper oxide to metallic copper.

For example, the operating conditions at which the flow cell is operated in step c) comprise current density ranging from -100 mA.cm² to -1.5 A.cm²; preferably from -150 mA.cm² to -1.0 mA.cm².

According to a **third aspect,** the disclosure provides the use of a system comprising a gas-fed flow cell with a bipolar membrane in a process for electrolysing carbon dioxide under acidic conditions in the presence of one or more alkali metal cations wherein the use further comprises an acidic catholyte having a pH of less than 5.5; with preference, the system is according to the second aspect and/or the process is according to the first aspect.

### Description of the figures

- **Figure 1** illustrates a system according to the disclosure.
- **Figure 2** illustrates a gas-fed flow cell according to the disclosure.
- **Figure 3** Schematic representation of different catholyte configurations and different membranes: a) alkaline bulk pH, where (bi)carbonate species accumulate in solution, b) acid bulk pH, where (bi)carbonate species are formed but are reconverted to CO₂ by protons in the bulk solution, c) proton exchange membrane (PEM), in which positively charged species can cross, resulting in unstable electrolyte composition over time and d) full cell assembly with a bipolar membrane (BPM), where (1) CO₂ is reduced to products, (2) CO₂ is converted to (bi)carbonate, (3) CO₂ is regenerated, (4) H₂O dissociates in the BPM interlayer, (5) protons diffuse into the catholyte allowing stable pH, (6) hydroxide ions diffuse into the anolyte allowing stable pH.
- **Figure 4** Results of the flow rate test concerning a) single-pass conversion and b) selectivity of the system. The data were obtained after performing each electrolysis for 30 min at -200 mA cm⁻² with a 0.05 M H₂SO₄ + 3 M KCI catholyte. a) Reducing the CO₂ flow rate enhances the SPC, which reaches a maximum of (29±3)% at 1.25 mL min⁻¹. b) Decreasing the flow rate from 10 to 1.25 mL min⁻¹ results in a selectivity loss for C₁ products in favour of C₂₊ products. The optimal flow rate is 1.25 mL min⁻¹, which provides high selectivity for C₂₊ species, 60%, and a good SPC value of (29 ± 3)%. These two parameters reach a plateau starting from 1 mL min⁻¹ due to excessive H₂ production, a result of scarce CO₂ availability in these conditions. The error bars represent the standard deviation of three measurements.
- **Figure 5** Results from the stability test performed at -200 mA cm⁻² with a CO₂ flow rate of 1.25 mL min⁻¹ and a 0.05 M H₂SO₄ + 3 M KCI catholyte: a) the selectivity remains constant, with ethylene FE around 30%, b) the BPM proves to be effective in keeping an elevated pH gradient through the cell for several hours, c) K⁺ monitoring through ICP-MS shows how the BPM is also able to stop K⁺ crossover, maintaining a concentration around 3 M (117 g L⁻¹) in the catholyte and 2.5 M (98 g L⁻¹) in the anolyte, d) the full cell potential (E_{full}) and SPC are both stable with values around -5.4 V and 26%, respectively.
- **Figure 6** Schematic representation of the two outlets of the reactor (a) and how CO₂ is distributed among them (b). The results were collected after 30 min electrolysis with a CO₂ flow rate of 1.25 mL min⁻¹ and a 0.05 M H₂SO₄ + 3 M KCI catholyte. a) CO₂ and gaseous products can be collected either at the direct outlet or from the indirect outlet. The CO₂ pathway to products is not shown for simplicity. (1) CO₂ that bypasses the cell without crossing the GDE, (2) CO₂ conversion to (bi)carbonate, (3) CO₂ regeneration, and (4) r-CO₂ that degasses from the solution and exits through the catholyte outlet. b) When no current is applied, most of the inlet CO₂ can be found at the gas outlet (93%), while during the electrolysis the majority is collected from the catholyte stream (66%). The main difference between the two situations is that in the first case the CO₂ never reacts, and in the latter what can be collected is essentially regenerated CO₂.
- **Figure 7** X-ray diffraction (XRD) diffractograms for the as-synthesized CuO nanoparticles (top) and the reduced Cu catalyst after activation (bottom).
- **Figure 8** Effects of varying concentrations of KCI in a 0.05 M H₂SO₄ electrolyte with a 10 mL min⁻¹ CO₂ inlet flow rate. When no KCI is present, CO₂ is not reduced and instead HER is predominant. 0.5 M of KCI is already enough to suppress H₂O reduction, but since 3 M yields the same product distribution with a less negative E_{cell}, we decided to choose this value for our catholyte.
- **Figure 9** Single-pass conversion as a function of the productivity of the reactor expressed in mg of CO₂ converted to reduction products per minute. The 30 min electrolysis was carried out in 0.05 M H₂SO₄ + 3 M KCI at -200 mA cm⁻² with increasing CO₂ inlet flow rate (from 1 to 10 mL min⁻¹, from left to right). The correlation shows a clear trade-off between conversion and productivity.
- **Figure** 10 Concentration of reactant (CO₂), intermediate (CO) and product (C₂H₄) as a function of single-pass conversion for an electrolysis at -200 mA cm⁻² with a CO₂ inlet flow rate of 1.25 mL min⁻¹. CO decreases while C₂H₄ increases in parallel with the SPC%, which in line with a series reaction that has CO as the intermediate. These concentrations comprise both the direct and indirect streams, and a purging argon flow of 35 mL min⁻¹ is taken in to account.

### Detailed description

For the disclosure, the following definitions are given:
The terms "comprising", "comprises" and "comprised of" as used herein are synonymous with "including", "includes" or "containing", "contains", and are inclusive or open-ended and do not exclude additional, non-recited members, elements, or method steps. The terms "comprising", "comprises" and "comprised of" also include the term "consisting of".

The recitation of numerical ranges by endpoints includes all integer numbers and, where appropriate, fractions subsumed within that range (e.g. 1 to 5 can include 1, 2, 3, 4, 5 when referring to, for example, a number of elements, and can also include 1.5, 2, 2.75 and 3.80, when referring to, for example, measurements). The recitation of endpoints also includes the recited endpoint values themselves (e.g. from 1.0 to 5.0 includes both 1.0 and 5.0). Any numerical range recited herein is intended to include all sub-ranges subsumed therein.

The disclosure provides a process for electrolysing carbon dioxide that includes CO₂ regeneration and recycling of said regenerated CO₂ back into the input flow. The disclosure also provides a system suitable for carbon dioxide electrolysis that comprises a gas-fed flow cell and means to recover CO₂ from the catholyte outlet and redirect it to the gas inlet. The process and the system will be described jointly by reference to Figures 1 and 2.

The disclosure provides **a process** for electrolysing carbon dioxide as defined in claim 1.

With preference, the indirect gas stream exiting from the catholyte reservoir comprises carbon dioxide, and the process further comprises a step e) of recovering the indirect gas stream exiting from the catholyte reservoir and recycling said indirect gas stream into the gas input flow comprising carbon dioxide of step d).

Indeed, it was found that the process allows obtaining an indirect gas stream that is composed of almost pure CO₂, which allows the reinjection in the cell without previous separation.

For example, the indirect gas stream exiting from the catholyte reservoir comprises at least 90 mol.% of CO₂ based on the total molar content of the indirect gas stream; preferably at least 95 mol.%; more preferably at least 98 mol.%.

The gas-fed flow cell 3 comprises a gas chamber 5, a catholyte chamber 7, and an anolyte chamber 9. For example, the gas chamber 5 has a gas channel 11, through which a gas flow comprising CO₂ is circulating. Gas chamber 5 comprises a gas inlet 13 and a gas outlet 15 and is separated from the catholyte chamber 7 by a gas diffusion electrode 17. The catholyte chamber 7 and the anolyte chamber 9 (when present) are separated by a membrane 19 which is selected to be a bipolar membrane. The gas-fed flow cell comprises a cathode (not represented). The gas-fed flow cell also comprises an anode 21, for example, a Ni foam anode, which is contained in the anolyte chamber or that is in direct contact with the membrane Any oxygen evolution reaction (OER) catalyst and anode compartment design can be used. In particular when anolyte is alkaline then non noble metal catalyst can be used.

With preference, the gas-fed flow cell comprises a reference electrode. It is preferred that said reference electrode is an Ag/AgCl electrode filled with KCI at a concentration ranging from 3.0 to 3.8 M; preferably from 3.2 to 3.6 M; even more preferably with 3.4 M of KCI. In other implementations of the invention, the reference electrode could also be a reversible hydrogen electrode (RHE).

Advantageously, the electrically conductive connection from the gas diffusion electrode 17 and the potentiostat is achieved by applying copper tape on said gas diffusion electrode 17, the copper tape being electrically connected to a metallic rod in contact with the potentiostat. For example, the metallic rod is a steel rod, preferably a stainless-steel rod.

The system is remarkable in that it comprises the catholyte being an acidic catholyte comprising one or more alkali metal cations and means to recover an indirect gas stream exiting the gas outlet of the catholyte reservoir and means to recycle the said indirect gas stream into the gas chamber.

Thus, the disclosure provides a system 1 suitable to perform the process of electrolysing carbon dioxide as defined in claim 14.

It is preferred that the system employs bipolar membranes (BPMs), operated in reverse bias mode, which permits the use of acidic catholyte with alkaline anolyte.

BPMs are composed of an anion exchange layer (AEL) coupled with a cation exchange layer (CEL), and function by carrying out water dissociation at the interlayer (IL) to transport protons toward the catholyte and hydroxide ions toward the anolyte (Figure 5d). This stabilizes pHs in each compartment and maintains a pH gradient, which avoids permanent (bi)carbonate formation at the cathode while also permitting the use of Earth-abundant OER catalysts that are stable in alkaline conditions. Additionally, the transport of cations, anions, and CO₂R products should be blocked by the membrane, limiting any negative effect of ion deposition at the cathode.

Although BPMs have recently shown promising results in alkaline systems and membrane electrode assemblies, they have so far not been implemented in acidic gas-fed flow cells. The disclosure discloses a BPM-based system incorporating an oxide-derived Cu catalyst, which achieves a high C₂₊ selectivity (> 60%) for acidic CO₂R. By assessing the composition of the gas outlets of the reactor, it was shown how carbonate species can be completely converted to r-CO₂, which is almost completely free of any products. Through analysis of selectivity, activity, and stability, it was highlighted some key advantages of bipolar membranes for high-rate CO₂R in acid at high conversions.

Thus, the gas-fed flow cell comprises a bipolar membrane separating the catholyte chamber from the anolyte chamber. The bipolar membrane includes a cation-exchange layer (CEL) and an anion-exchange layer (AEL), wherein the cation-exchange layer is in cation communication with the catholyte to provide protons into the catholyte and the anion-exchange layer is in anion communication with the anolyte. In other words, the bipolar membrane is used to dissociate water, thereby providing hydroxide ions to the anolyte chamber and protons to the catholyte chamber. The use of a bipolar membrane allows an asymmetric set up allowing the use of acidic catholyte with alkaline anolyte. Thus, the catholyte pH is less than the anolyte pH and step b) of the process comprises providing a catholyte flow and an anolyte flow wherein the catholyte pH is less than the anolyte pH.

As shown in Figure 3a, the gas diffusion electrode 17 of the present disclosure has a gas diffusion membrane 37 and further comprises an ink 39 deposited on the gas diffusion membrane 37; wherein the ink 39 comprises an ion-conducting polymer and a metal-based catalyst. The metal of the metal-based catalyst is preferably selected from copper, silver, and any mixture thereof. In a preferred embodiment, the metal-based catalyst is or comprises copper oxide nanoparticles.

Thus, in a preferred embodiment, step (a) of providing a system comprising a gas-fed flow cell comprises preparing said gas-fed flow cell by spray-coating an ink 39 comprising an ion-conducting polymer and a metal-based catalyst on a gas diffusion membrane 37.

For example, the metal-based catalyst is or comprises copper oxide nanoparticles and the process comprises a catalyst activation step to reduce copper oxide to metallic copper.

The gas diffusion membrane 37 allows for the diffusion of carbon dioxide as the main reactant of the electrolysis reaction into the electrochemical cell and is preferably hydrophobic porous support. In gas-fed flow cell 3, the gas diffusion membrane 37 is comprised within the gas chamber 5 of said gas-fed flow cell 3. With preference, said support shows a pore size ranging from 400 nm to 500 nm as determined by scanning electron microscopy, preferably from 420 nm to 580 nm or from 440 nm to 560 nm. The gas diffusion membrane is preferably selected from an ion-conducting polymer-based membrane, an ion-conducting inorganic material, a combination polymer/inorganic based membrane, and the like.

It is preferred that the gas diffusion membrane is a hydrophobic, porous, and chemically inert support. For example, the gas diffusion membrane 37 is or comprises polytetrafluoroethylene (PTFE). Examples of suitable membranes are commercially available from Fisher Scientific SAS under the commercial denomination Sartorius.

With preference, the gas diffusion membrane 17 has a circular shape and/or has a surface area of at least 1 cm² or at least 2 cm². For example, the gas diffusion membrane 17 has a thickness ranging from 2 µm to 50 µm measured by scanning electron microscopy, preferably from 5 µm to 40 µm, more preferably from 8 µm to 30 µm.

An ink 39 is deposited on the gas diffusion membrane 37 and comprises an ion-conducting polymer. With preference, the ion-conducting polymer is or comprises an ionomer. For example, the ion-conducting polymer is or comprises an ionomer with a tetrafluoroethylene backbone group (-CF2-CF2-). Such ionomers are capable of creating strongly hydrophobic nanoporous networks. For example, said ion-conducting polymer is or comprises a perfluorinated sulfonic acid, such as Nafion^{®} (tetrafluoroethylene-perfluoro-3,6-dioxa-4-methyl-7-octenesulfonic acid copolymer); and/or the ion-conducting polymer is or comprises tetrafluoroethylene-perfluoro(3-hydrophobioxa-4-pentenesulfonic acid) copolymer, such as Aquivion^{®}.

The ink can form a layer on the gas diffusion membrane, said layer having a thickness ranging from 2 nm and 100 µm measured by transmission electron microscopy, preferably from 4 µm and 10 µm, more preferably from 5 µm and 8 µm. In a preferred embodiment, the ink is deposited on the gas diffusion membrane by spray-coating.

For example, ink 19 has a ratio of the copper oxide nanoparticles over the ion-conducting polymer. With preference, the ink has a ratio of the copper oxide nanoparticles over the ion-conducting polymer ranging from 0.1 to 10 µL of ion-conducting polymer for 1 mg of catalyst (1:1).

For example, the gas diffusion electrode 17 has a mass loading of the ink 39 onto said gas diffusion membrane 37 ranging from 0.50 mg/cm² to 4.00 mg/cm², preferably from 1.50 mg/cm² to 3.00 mg/cm²; and more preferably from 2.00 mg/cm² to 2.50 mg/cm². The mass loading can be determined by weighing before and after deposition and drying.

In a preferred embodiment, the metal-based catalyst is provided in the form of nanoparticles having an average diameter ranging from 5 nm to 200 nm as measured by transmission electron microscopy, preferably from 10 nm to 150 nm, more preferably from 20 nm to 100 nm.

For example, the copper oxide nanoparticles have an average diameter ranging from 5 nm to 200 nm as measured by transmission electron microscopy, preferably from 10 nm to 150 nm, more preferably from 20 nm to 100 nm.

In a preferred embodiment, the gas input flow provided in step (d) has a flow rate of at most 10 mL/min; preferably, at most 5 mL/min; more preferably at most 3.5 mL/min; even more preferably at most 3.0 mL/Min; most preferably at most 2.8 mL/min; and even most preferably at most 2.5 mL/min or at most 1.8 mL/min. Indeed, as demonstrated in the example section, it was found that operating at a low flow rate of CO₂ enhances the single-pass conversion to multicarbon CO₂R products (SPC).

For example, the gas input flow provided in step (d) has a flow rate of at least 0.5 mL/min; preferably of at least 0.6 mL/min; more preferably of at least 0.7 mL/min; even more preferably of at least 0.8 mL/Min; most preferably of at least 0.9 mL/min; and even most preferably of at least 1.0 mL/min or at least 1.1 mL/min. Indeed, as demonstrated in the example section, it was found that operating at a too low flow rate enhances H₂ production. It is understood that the above values are given for a cell wherein the dimensions are 7.5cm x 7.5 cm x 3.2 cm. These values will be adapted by the person skilled in the art without difficulties in case the dimensions of the cell are changed.

For example, the gas input flow provided in step (d) has a flow rate ranging from 0.5 to 10 mL/min; preferably from 0.6 to 5 mL/min; more preferably from 0.7 to 3.5 mL/min; even more preferably from 0.8 to 3.0 mL/Min; most preferably from 0.9 to 2.8 mL/min; and even most preferably from 1.0 to 2.5 mL/min or from 1.1 to 1.8 mL/min.

Thus, it is preferred that the system further comprises a mass flow controller that is operatively connected to the gas chamber inlet to adjust an inlet gas flow rate.

For example, the gas input flow provided in step (d) comprises at least 3 mol% of carbon dioxide based on the total molar content of the input flow; preferably at least 20 mol% of carbon dioxide, more preferably at least 50 mol% of carbon dioxide
In a preferred embodiment, the gas input flow provided in step (d) comprises at least 85 mol% of carbon dioxide based on the total molar content of the input flow; preferably at least 90 mol% of carbon dioxide, more preferably at least 95 mol% of carbon dioxide; and even more preferably at least 98 mol%. For example, the gas input flow further comprises N₂.

In a preferred embodiment, the acidic catholyte has a pH of at most 5.4; preferably of at most 5.2; more preferably, of at most 5.0; even more preferably of at most 4.8or of at most 4.6; most preferably of at most 4.5 or of at most 4.2; even most preferably of at most 4.0 or of at most 3.5.

For example, the acidic catholyte has a pH of at least 0.5; preferably of at least 0.6; more preferably, of at least 0.7; even more preferably of at least 0.8 or at least 0.9; most preferably of at least 1.0 or above 1.0; even most preferably of at least 1.1.

For example, the acidic catholyte has a pH ranging from 0.5 to less than 5.5 or from 0.5 to 5.4; preferably from 0.6 to 5.2; more preferably from 0.7 to 5.0; even more preferably from 0.8 to 5.4 or from 0.8 to 5.0; most preferably from 0.9 to 4.5; even most preferably from 1.0 to 4.0 or from 1.1 to 3.5.

For example, the acidic catholyte comprises one or more acids at a concentration ranging from 0.001 to 5.0 M; preferably from 0.005 to 3.0 M or from 0.01 to 2.0 M; or from 0.05 to 1.5 M or from 0.01 to 1.0 M.

In an embodiment, the acidic catholyte comprises one or more acids at a concentration ranging from 0.001 to 5.0 M and one or more alkali metal cation donors at a concentration ranging from 0.5 to 5.0 M.

For example, the cations are weakly hydrated cations, and/or the alkali metal cations are one or more selected from Cs+, K+, Li+, and Na+; preferably the one or more alkali metal cations are or comprise K+.

For example, the acidic catholyte comprises one or more alkali metal cation donors selected from caesium chloride, caesium iodide, caesium sulfate, caesium phosphate, caesium hydroxide, potassium chloride, potassium phosphate monobasic, potassium sulfate, potassium iodide, potassium hydroxide, lithium chloride, lithium iodide, lithium sulfate, lithium phosphate, lithium hydroxide, sodium chloride, sodium sulphate, sodium iodide, sodium phosphate, and sodium hydroxide; preferably selected from potassium chloride, potassium phosphate monobasic, potassium sulfate, potassium iodide, and potassium hydroxide; more preferably the one or more alkali metal cation donors are or comprise potassium chloride.

With preference, the one or more alkali metal cation donors at a concentration ranging from 0.5 to 5.0 M; preferably ranging from 1.0 to 4.5 M; and more preferably ranging from 2.0 to 4.0 M.

In an embodiment, the acidic catholyte comprises one or more acids selected from hydrochloric acid, sulfuric acid, hydrobromic acid, hydriodic acid, perchloric acid, and chloric acid; preferably sulfuric acid.

For example, the one or more acids are present at a concentration ranging from 0.01 to 1.0 M; preferably, from 0.02 to 0.5 M; more preferably ranging from 0.03 to 0.2 M.

For example, the anolyte is an aqueous solution of one or more inorganic bases having a concentration ranging from 1 M to 10 M; preferably from 3 to 7 M or from 5 M to 10 M. For example, the aqueous solution of one or more inorganic bases has a concentration that is at least 5 M. With preference, the anolyte has a pH ranging from 7 to 15; preferably from 10 to 14.

With preference, the one or more inorganic bases are alkali selected from NaOH, KOH, Ca(OH)₂, LiOH, Mg(OH)₂, RbOH, CsOH, and any mixture thereof. With preference, the one or more inorganic bases are or comprise KOH and/or NaOH.

The system preferably comprises one or more peristaltic pumps operatively connected to a first tube in fluid communication with the anolyte chamber to circulate the anolyte therein, and to a second tube in fluid communication with the catholyte chamber to circulate the catholyte therein. It is preferred that the catholyte and anolyte are circulated at a constant flow rate. For example, the catholyte flow rate is around 25 mL/min, while the anolyte flow rate is around 5.5 mL/min
In an embodiment the operating conditions at which the flow cell is operated in step c) comprise current density ranging from -100 mA.cm² to -1.5 A.cm²; preferably ranging from - 120 mA.cm² to -1.2 A.cm²; more preferably from -150 mA.cm² to -1.0 A.cm².

In an embodiment the operating conditions at which the flow cell is operated in step c) comprises a voltage ranging from -1,7 V to -7 V; preferably ranging from -3.5 V to -6 V and more preferably from -4.5 V to -5.5 V.

Thus, the system further comprises a power source providing electric current at an applied current density.

### Test Methods

Mass loading of the ink onto the gas diffusion membrane: The membrane was weighed using an analytical balance before deposition and after drying overnight in a vacuum desiccator.

Transmission Electron Microscopy: TEM analysis was conducted using a Jeol 2100F microscope equipped with Schottky Field Emission electron gun and an ultra-high resolution polar piece.

Scanning Electron Microscopy: SEM images were obtained using a SU-70 Hitachi FEG-SEM.

X-Ray Diffraction: XRD data were obtained from a D8 ADVANCE diffractometer (Bruker) using a Cu Kα X-ray source (1.5406Å). Peaks were attributed using the PDF-2/release 2013 RDB database.

Nuclear Magnetic Resonance: Liquid products were analysed using ¹H NMR with a presaturation water suppression method on a Bruker Advance III 300 MHz spectrometer at 300 K. D₂O was used as the lock solvent and an aqueous solution of terephthalic acid was used as an internal standard for quantification.

Inductively Coupled Plasma Mass Spectrometry: The quantification of K⁺ was performed with a Nexion 2000B inductively coupled plasma atomic mass spectrometer (Perkin-Elmer) using the Syngistix^{™} software.

Gas products were detected on-line using an SRI instruments 8610 GC with Ar as the carrier gas. The GC was fitted with a thermal conductivity detector for H2 quantification, where the gas was separated using a HaySepD precolumn with a 3 m molecular sieve column. Carbon products were separated using a 5 m HaySepD column (CO, C2H4) and detected using a flame-ionization detector fitted with a methanizer. Calibration was performed using a custom standard gas mixture in CO2.

The FE for gas products was calculated using equation 1: $FE \left(%\right) = \frac{{n}_{product} \times {n}_{electrons} \times F}{\left({Q}_{t = 0}-{Q}_{t = x}\right)}$

Where n_{produc}t is the amount of product obtained (mol), n_{electrons} is the number of electrons used to make the product, F is the Faraday constant (C mol-1), Qₜ₌₀ is the charge at the time of the injection, and Qₜ₌ₓ is the charge at time x seconds before the injection, representing the time taken to fill the sample loop, with x depending on the combined flow rate of Ar and CO₂ as well as the loop size.

### Liquid Product Analysis

Liquid products were analysed using ¹H NMR with a presaturation water suppression method on a Bruker Advance III 300 MHz spectrometer at 300 K. D2O was used as the lock solvent and an aqueous solution of terephthalic acid was used as an internal standard for quantification. The product crossover through the bipolar membrane was accounted for by liquid sampling from the anode compartment

### Electrolyte Analysis

The quantification of K⁺ was performed with a Nexion 2000B inductively coupled plasma atomic mass spectrometer (Perkin-Elmer) using the Syngistix^{™} software.

### Single-Pass Conversion Calculations

The single-pass conversion was calculated for each product using equation 2: $SPC % = \left[\left(\frac{{j}_{product} \times 60 s}{{n}_{electrons} \times F}\right)\div \left(\frac{flow rate}{24.05 L}\right)\right] \times carbon atoms \times 100$ Where j_{product} is the partial current density for a particular product (mA cm⁻²), n_{electrons} is the number of electrons needed for the reduction, F is the Faraday constant (C mol⁻¹), the flow rate is the one chosen for CO₂ (L min⁻¹), and 24.05 L equals to the molar volume of a gas at NTP. The total SPC% is obtained by adding the individual SPC% together.

### Productivity Calculations

The productivity (P, in mg of reduced CO₂ min⁻¹ cm⁻²) was calculated for each CO₂ inlet flow rate value according to equation 3: $P = {mm}_{CO 2} \times \frac{{CO}_{2 red}}{{t}_{GC}} \times 1000$ Where mm_{CO2} is the molar mass of CO₂ (g mol⁻¹), CO_{2 red} is the amount of reduced CO₂ (mol) and t_{GC} is the time needed to fill the GC loop (min) with a specific CO₂ inlet flow rate. The GC loop volume (0.5 mL) is the unit used to quantify the amounts of CO₂ and products.

### Examples

### Example 1: synthesis of the catalyst and preparation of the gas diffusion electrodes

A CuO catalyst was synthesized using a simple solvothermal procedure as described in Z. Shan Hong, Y. Cao, J. fa Deng, Mater. Lett. 2002, 52, 34-38.

In brief, a solution of Cu(acetate)₂ in ethanol was heated to 200 °C in an autoclave for 20 h to obtain nanoparticles approximately 50 nm in size.

Gas diffusion electrodes (GDEs) were formed by spray-coating an ink being a methanolic solution containing CuO nanoparticles and Nafion^{®} (tetrafluoroethylene-perfluoro-3,6-dioxa-4-methyl-7-octenesulfonic acid copolymer) onto a polytetrafluoroethylene (PTFE) membrane to reach a loading of 2 mg cm⁻², corresponding to an approximate thickness of 6 µm
An activation step was required to obtain metallic Cu from the initial oxide, which involved running consecutive linear sweep voltammograms (LSVs) from 0.1 V to -1 V vs. RHE until the response was constantly followed by chronopotentiometry (CP) at -200 mA for 1 h using a 3 M KCI solution as the catholyte (XRD in figure 7). These activated Cu-GDEs were used for all experiments.

### Example 2 - Electrochemical experiments

The anolyte (2.5 M KOH, pH 14) was kept constant throughout all experiments and only the catholyte composition was varied. A catholyte comprising H₂SO₄ (0.05 M, pH 1) was selected and the effects arising from the addition of varying amounts of KCI were explored. As expected, the addition of KCI improved selectivity by limiting H₂ evolution (Figure 8). The high conductivity of the electrolyte salt also reduced the solution resistance, thereby lowering the full cell potential. With 3 M KCI, a high C₂₊ product selectivity (52%) and a low cell potential (-4.7 V, -200 mA cm⁻²) were achieved.

A parameter employed to showcase and evaluate the cell performance is the single-pass CO₂ conversion to CO₂R products (SPC), which describes the yield of CO₂R products, see below equation 3. $SPC % = \left\{\left[\left(\frac{{j}_{product} \times 60 s}{{n}_{electrons} \times F}\right)+\left(\frac{flow rate}{molar volume}\right)\right]\times carbon atoms\times 100\right\}$

In equation 3, j_{product} is the partial current density for a specific product (mA cm⁻²), n_{electrons} is the number of electrons needed for the reduction, F is the Faraday constant, the flow rate is the one chosen for the inlet CO₂ (mL min⁻¹), and 24.05 L equals to the molar volume of a gas at normal temperature and pressure. Several factors can alter the SPC including the reaction rate, the flow rate of CO₂, and the type and amount of products generated. This is because the product influences the amount of hydroxide ions formed, which in turn will determine how much CO₂ is converted to transient (bi)carbonate species (see Eq. 1-2). In an ideal reactor with complete selectivity for CO, two OH⁻ are formed for every molecule of product. Consequently, only 50 % of the input CO₂ (i.e., CO₂ in) can be converted to reduction products. Similarly, in the case of a catalyst selective only towards ethylene twelve OH⁻ are generated per molecule of ethylene formed, resulting in a maximum ethylene yield of only 25% (see eq. 4 and 5). This results in the SPC being heavily dependent on the fate of the r-CO₂ (equation 3).

CO₂ + H₂O + 2e⁻ ⇄ CO + 2 OH⁻ (Equation 4)

2 CO₂ + 8 H₂O + 12 e⁻ ⇄ C₂H₄ + 12 OH⁻ (Equation 5)

These effects were explored by altering the CO₂ inlet flow rate at a fixed current density of -200 mA cm⁻². As expected, decreasing the flow rate increased the SPC to reach a high SPC value of (29 ± 3) % at 1.25 mL min⁻¹ (Figure 4a). Lowering the flow rate to 1 mL min⁻¹ does not lead to a better SPC, which plateaus around 29%; instead, the Faradaic efficiencies (FEs) of CO₂R products decrease while hydrogen production becomes dominant. This loss in CO₂R selectivity at 1 mL min⁻¹ represents the region in which all CO₂ is either converted to CO₂R products or (bi)carbonate. Hence, due to the scarcity of CO₂, the surplus current density is mainly used for water reduction to H₂, which leads to poor selectivity.

Interestingly, it was observed an increase in C₂₊ Faraday efficiency with a decreasing flow rate of CO₂ at the expense of C₁ products (Figure 4b). High FEs for ethylene, (34 ± 4) %, and ethanol, (22 ± 3) %, were obtained at 1.25 mL min⁻¹. To help rationalize this, the CO₂, C₁, and C₂₊ concentrations were plotted as a function of conversion (see figures 9 and 10), which shows that the concentrations for C₁ products are decreasing while those for C2+ products increase in parallel to conversion. This concentration profile is typical for a series reaction and in line with the conversion of CO₂ to C₂₊ products via CO as an intermediate (see T. K. Todorova, M. W. Schreiber, M. Fontecave, ACS Catal. 2020, 10, 1754-1768.).

At low conversions CO₂ concentrations and hence CO₂ coverage of active sites are high, resulting in the formation of mainly primary C1 products. With increasing conversions, however, CO₂ concentrations are reduced while CO concentrations are increased alongside their respective coverage on active sites, resulting in an increasing Faraday efficiency for secondary C₂₊ products. This increase in Faraday efficiency alongside conversion is likely to be amplified by C₂₊ formation from CO which is probably a second-order reaction.

At high conversions, most of the CO₂ seems to be directly converted to C₂₊ products and not to the C₁ product formate, inert to further electroreduction. This hints at the reaction rate of C₂₊ formation being considerably higher compared to the reaction rate of formate formation at high conversions.

The ability of the electrolyser to operate at high conversion over extended periods was assessed. Over 8 h, the FEs for CO₂R products were stable and, through analysis of liquid samples from the anolyte using ¹H NMR, it was confirmed that there was no product crossover between the cell compartments. Additionally, it was shown that a stable catholyte pH could be maintained for the duration of the experiment even with an alkaline anolyte. Inductively coupled plasma-mass spectroscopy (ICP-MS) was used to detect any crossover of K⁺ and it was observed that there is no significant shift in K⁺ concentration on either side of the cell. The system could keep a constant full cell potential (E_{cell}) of -5.4 V with an average SPC of 26% towards CO₂R products.

The stability of the electrolyte in terms of pH and K⁺ concentration highlights two clear benefits of the BPM. However, this kind of membranes introduces a voltage penalty due to water dissociation at the IL, which thermodynamic value is 0.83 V in our case and changes depending on the pH gradient between the cell compartments. This is why the reactor reaches the high E_{cell} value of -5.4 V. Despite this disadvantage, recent progress in catalyst-loaded BPMs opens ways to keep the many benefits of bipolar membranes while avoiding the negative voltage contribution.

With the system employed, if the r-CO₂ were to completely re-react on the copper surface to form products, it would be possible to achieve 100% SPC with the appropriate flow rate at a given current. However, this was not the case as the scarce availability of CO₂ at flow rates lower than 1.25 mL min⁻¹ leads to a trade-off in FE with more H₂ generation. Additionally, the r-CO₂ in the electrolyte is not expected to re-react on the copper NPs, since the high OH⁻ concentration at the catalyst surface would convert CO₂ to (bi)carbonate once again, therefore the CO₂ is more likely to degas through the catholyte solution. Considering this observation and the delicate dependency of the SPC on the product distribution, its value does not entirely reflect the CO₂ conversion efficiency of the system.

Thus, instead of striving to achieve high SPC values, having an elegant way of recovering and potentially recycling the CO₂ lost as carbonate seems more important. As a consequence, the composition of the different gas outlets of the reactor is highly important when identifying the best recycling method for the r-CO₂.

There are two gas outlets in the system. The first one is positioned at the back of the GDE and is identified as the direct outlet, which collects the unreacted CO₂ and the gas products. The other one is located in the catholyte reservoir and is termed as the indirect outlet, which collects the (r-)CO₂ and gas products that come from the solution. The streams coming out from both outlets under CO₂R conditions were analysed as well as under non-catalytic conditions to better understand the CO₂ distribution.

Firstly, we checked the amount of CO₂ passing through each exit point under idle conditions (0 mA cm⁻²) and under operating conditions (-200 mA cm⁻²) while keeping the inlet CO₂ flow rate constant at 1.25 mL min⁻¹ (Figure 6b). In both cases, the total amount of CO₂ and CO₂R products was the same, therefore providing a closed carbon mass balance. With no current, the majority of the inlet CO₂ (93%) was retrieved at the direct outlet. In contrast, under operating conditions, only a small fraction of inlet CO₂ (2%) was obtained at the direct outlet, while the rest, which is all r-CO₂, was found in the gas from the catholyte stream (66%).

This distribution shows that during electrolysis almost all of the inlet CO₂ crosses the GDE and is converted to either reduction products, which account for 32% of the inlet CO₂, in line with a SPC value of 29%, or (bi)carbonate. Then, the (bi)carbonate species are completely neutralized to regenerate CO₂, which exits the system preferentially through the indirect outlet. The composition of both streams showed that all the carbon gas products are obtained at the direct outlet, and only small quantities of hydrogen are seen in the indirect outlet stream alongside the r-CO₂. Consequently, the indirect stream can potentially be collected and readily recycled through the electrolyzer CO₂ inlet, where the CO₂ would be available to react again while H₂ and CO₂R products leave the electrolyzer via the direct outlet as a concentrated gas flow, elegantly avoiding downstream CO₂/products separation through processes such as amine-based capture, which typically dominates the energy consumption of the product purification. As devices move towards commercial operation at high conversions, cell modifications to improve gas management and CO₂ recovery will become highly important. Here we show that in this cell design and setup, independent of the used membrane, simple recovery would benefit overall device performance.

In conclusion, the CO₂R system of the disclosure shows high C₂₊ selectivity and good SPC that allows an easy recycling of CO₂. This result was obtained thanks to a combination of acid catholyte, which promotes the regeneration of CO₂ from carbonate, and low CO₂ inlet flow rate, which enhances the SPC and multicarbon products selectivity.

The optimized system, running at -200 mA cm⁻² with a CO₂ flow rate of 1.25 mL min⁻¹, can achieve satisfying results, with an SPC value of (29 ± 3) % and a C₂₊ product FE of 60%. In addition, it was able to recover an almost pure stream of r-CO₂ from the indirect outlet of the reactor, which opens the possibility of direct recycling avoiding the energy-intensive CO₂ separation from the products. At the same time, the direct outlet gives a flow of concentrated products with very little CO₂ content. The integration of a BPM in the reactor allows the use of inexpensive OER catalysts, other than opening the possibility for oxidation reactions requiring a lower overpotential and yielding more valuable products than O₂.

Results are reported in the below tables

**Table S1. Faradaic efficiencies and single-pass conversion values corresponding to the different inlet flow rates of CO₂ tested at -200 mA cm⁻².**

| | | **Faradaic Efficiency / %** | | | | | | |
|---|---|---|---|---|---|---|---|---|
| **Q / mL min⁻¹** | **E_{cell}** / **V** | **H₂** | **CO** | **C₂H₄** | **HCOOH** | **C₂H₅OH** | **C₃H₇OH** | **SPC%** |
| 10 | -5.3 ± 0.3 | 16.7 ± 2.5 | 14.7 ± 2.7 | 22.8 ± 6.5 | 18.6 ± 5.8 | 11.5 ± 3.1 | 5 ± 0.3 | 7 ± 0.8 |
| 5 | -5.4 ± 0.1 | 15.3 ± 0.7 | 11.8 ± 3.6 | 25.4 ± 5.4 | 17 ± 6.1 | 13 ± 4.1 | 5.5 ± 0.9 | 13.7 ± 1.1 |
| 2.5 | -5.5 ± 0.2 | 15.4 ± 0.6 | 9.9 ± 1.8 | 29.6 ± 3.9 | 14.3 ± 3.3 | 15.7 ± 2.1 | 6.3 ± 0.2 | 23.7 ± 2.1 |
| 1.25 | -5.5 ± 0.3 | 23.9 ± 2.9 | 1.6 ± 0.6 | 34.3 ± 4 | 2.6 ± 0.6 | 22 ± 2.8 | 3.7 ± 1.1 | 29.1 ± 2.6 |
| 1 | -5.6 ± 0.3 | 34.2 ± 3.5 | 1.1 ± 0.3 | 29.6 ± 3 | 1.6 ± 0.5 | 19.1 ± 2.8 | 1.8 ± 1 | 29.4 ± 3.7 |

**Table S2. Faradaic efficiencies and single-pass conversion values for the 8 h long electrolysis at -200 mA cm⁻² with an inlet CO₂ flow rate of 1.25 mL min⁻¹.**

| | **Faradaic Efficiency / %** | | | | | | |
|---|---|---|---|---|---|---|---|
| **Time / h** | **H₂** | **CO** | **C₂H₄** | **HCOOH** | **C₂H₅OH** | **C₃H₇OH** | **SPC%** |
| 1 | 32.5 | 1.8 | 32.5 | 2.4 | 23 | 1 | 27.2 |
| 2 | 34.1 | 1.7 | 31.4 | 2.1 | 19 | 4.8 | 26.5 |
| 3 | 37.1 | 1.7 | 30.6 | 2.2 | 21.1 | 3.6 | 26.8 |
| 4 | 35.2 | 1.6 | 31 | 2.6 | 21.2 | 3.7 | 27.4 |
| 5 | 36.6 | 1.6 | 30.2 | 2 | 17.3 | 2.8 | 24.4 |
| 6 | 37.1 | 1.6 | 29.7 | 2 | 20.5 | 2.9 | 25.5 |
| 7 | 37.9 | 1.6 | 29.7 | 2 | 18.8 | 3.1 | 24.8 |
| 8 | 38.4 | 1.5 | 29.7 | 2 | 20.2 | 2.9 | 25.3 |

**Table S3. Amounts of CO₂ found in the direct and indirect outlets with the fraction converted to CO₂R products.**

| | **CO₂ in direct outlet (nmol/s)** | **CO₂ in indirect outlet (nmol/s)** | **CO₂ to products (nmol/s)** |
|---|---|---|---|
| **0 mA cm⁻²** | 705.7 | 49 | - |
| **-200 mA cm⁻²** | 12.4 | 496.4 | 240.1 |

## Claims

1. Process for electrolysing carbon dioxide, said process is **characterized in that** it comprising the following steps:
a) providing a system comprising a gas-fed flow cell comprising a gas chamber with a gas inlet, a gas outlet, a catholyte chamber, and a gas diffusion electrode comprising a metal-based catalyst, wherein the gas diffusion electrode is placed between the gas chamber and the catholyte chamber;
b) providing a catholyte flow and an anolyte flow into said gas-fed flow cell;
c) activating said gas-fed flow cell under operating conditions;
d) providing a gas input flow comprising carbon dioxide using the gas inlet of the gas chamber to produce a direct gas stream exiting from the gas outlet of the gas chamber and a liquid catholyte output flow from the catholyte chamber comprising products, wherein said liquid catholyte output flow is degassing in a catholyte reservoir to produce an indirect gas stream exiting from a gas outlet of the catholyte reservoir;
wherein the catholyte flow is an acidic catholyte flow comprising one or more alkali metal cations and **in that** the gas-fed flow cell comprises a bipolar membrane includes a cation-exchange layer in contact with the catholyte and an anion-exchange layer in contact with the anolyte; wherein the cation-exchange layer provides protons to the catholyte and the anion exchange layer provides hydroxide ions to the anolyte; **in that** the acidic catholyte has a pH of at most 5.5 and **in that** the catholyte pH is less than the anolyte pH.

2. The process according to claim 1 is **characterized in that** the indirect gas stream exiting from the catholyte reservoir comprises carbon dioxide, and **in that** the process further comprises a step e) of recovering the indirect gas stream exiting from the catholyte reservoir and recycling said indirect gas stream into the gas input flow comprising carbon dioxide of step d).

3. The process according to claim 1 or 2 is **characterized in that** the gas input flow provided in step (d) has a flow rate ranging from 0.5 to 10 mL/min; preferably from 0.9 to 2.8 mL/min or from 1.0 to 2.5 mL/min.

4. The process according to any one of claims 1 to 3 is **characterized in that** the acidic catholyte has a pH ranging from 0.5 to 5.4; preferably from 1.0 to 4.0.

5. The process according to any one of claims 1 to 4 is **characterized in that** the anolyte has a pH ranging from 7 to 15; preferably from 10 to 14.

6. The process according to any one of claims 1 to 5 is **characterized in that** the acidic catholyte comprises one or more acids at a concentration ranging from 0.01 to 1.0 M and one or more alkali metal cation donors at a concentration ranging from 1.0 to 5.0 M.

7. The process according to claim 6 is **characterized in that** the one or more alkali metal cations are one or more selected from Cs⁺, K⁺, Li^{+,} and Na⁺; preferably the one or more alkali metal cations are or comprise K⁺.

8. The process according to any one of claims 1 to 7 is **characterized in that** the acidic catholyte comprises one or more alkali metal cation donors selected from caesium chloride, caesium iodide, caesium sulfate, caesium phosphate, caesium hydroxide, potassium chloride, potassium phosphate monobasic, potassium sulfate, potassium iodide, potassium hydroxide, lithium chloride, lithium iodide, lithium sulfate, lithium phosphate, lithium hydroxide, sodium chloride, sodium sulphate, sodium iodide, sodium phosphate and sodium hydroxide; preferably selected from potassium chloride, potassium phosphate monobasic, potassium sulfate, potassium iodide, and potassium hydroxide; more preferably the one or more alkali metal cation donors are or comprise potassium chloride.

9. The process according to claim 8 is **characterized in that** the one or more alkali metal cation donors at a concentration ranging from 0.5 to 5.0 M; preferably ranging from 2.0 to 4.0 M.

10. The process according to any one of claims 1 to 9 is **characterized in that** the acidic catholyte comprises one or more acids selected from hydrochloric acid, sulfuric acid, hydrobromic acid, hydriodic acid, perchloric acid, and chloric acid; preferably sulfuric acid.

11. The process according to claim 10 is **characterized in that** the one or more acids are present at a concentration ranging from 0.01 to 1.0 M; preferably, from 0.02 to 0.5 M; more preferably ranging from 0.03 to 0.2 M.

12. The process according to any one of claims 1 to 11 is **characterized in that** the metal of the metal-based catalyst is selected from copper, silver and any mixture thereof; and/or the metal-based catalyst is or comprises copper oxide nanoparticles and the process comprises a catalyst activation step to reduce copper oxide to metallic copper.

13. The process according to any one of claims 1 to 12 is **characterized in that** the operating conditions at which the flow cell is operated in step c) comprise current density ranging from -100 mA.cm² to -1.5 A.cm²; preferably from -150 mA.cm² to -800 mA.cm².

14. A system (1) suitable to perform the process for electrolysing carbon dioxide according to any one of claims 1 to 13, the system comprising a gas-fed flow cell (3) comprising a gas chamber (5), a catholyte chamber (7) and an anolyte chamber (9), wherein said gas chamber (5) is separated from the catholyte chamber (7) by a gas diffusion electrode (17), said gas diffusion electrode (17) having a gas diffusion membrane being comprised within said gas chamber, wherein said catholyte chamber (7) and said anolyte chamber (9) comprise respectively a cathode and an anode, and wherein the system (1) further comprises catholyte (23) and anolyte (25) and means (27; 29) to flow the catholyte (23) and the anolyte (25) within respectively said catholyte chamber (7) and said anolyte chamber (9);
wherein the system is **characterized in that** the catholyte flow is an acidic catholyte flow comprising one or more alkali metal cations and **in that** the gas-fed flow cell comprises a bipolar membrane (19) that includes a cation-exchange layer in contact with the catholyte and an anion-exchange layer in contact with the anolyte; wherein the cation-exchange layer provides protons to the catholyte and the anion exchange layer provides hydroxide ions to the anolyte; **in that** the acidic catholyte has a pH of at most 5.5 and **in that** the catholyte pH is less than the anolyte pH;
and wherein the system (1) further comprises a catholyte reservoir to receive and degas the liquid catholyte output flow exiting the catholyte chamber, and with preference, means (31) to recover an indirect gas stream exiting the gas outlet (33) of the catholyte reservoir, and means (35) to recycle the said indirect gas stream back into the gas chamber (5).

15. Use of a system comprising a gas-fed flow cell (3) with a bipolar membrane (19) in a process for electrolysing carbon dioxide under acidic conditions in the presence of one or more alkali metal cations; wherein the system is according to claim 14 and/or the process is according to any one of claims 1 to 13.

## Patentansprüche

1. Verfahren zur Elektrolyse von Kohlendioxid, wobei das Verfahren **dadurch gekennzeichnet ist, dass** es die folgenden Schritte umfasst:
a) Bereitstellung eines Systems, das eine gasgespeiste Durchflusszelle umfasst, welche eine Gaskammer mit einem Gaseinlass, einem Gasauslass und einer Katholytkammer sowie eine Gasdiffusionselektrode mit einem Katalysator auf Metallbasis umfasst, wobei die Gasdiffusionselektrode zwischen der Gaskammer und der Katholytkammer angeordnet ist;
b) Zuführen eines Katholytstroms und eines Anolytstroms in die mit Gas versorgte Durchflusszelle;
c) Aktivieren der gasgespeisten Durchflusszelle unter Betriebsbedingungen;
d) Zuführen eines Gaseinlassstroms, der Kohlendioxid enthält, über den Gaseinlass der Gaskammer, um einen direkten Gasstrom zu erzeugen, der aus dem Gasauslass der Gaskammer austritt, sowie eines flüssigen Katholyt-Auslassstroms aus der Katholytkammer, der Produkte enthält, wobei der flüssige Katholyt-Auslassstrom in einem Katholytbehälter entgast wird, um einen indirekten Gasstrom zu erzeugen, der aus einem Gasauslass des Katholytbehälters austritt;
wobei der Katholytenstrom ein saurer Katholytenstrom ist, der ein oder mehrere Alkalimetallkationen enthält, und wobei die mit Gas gespeiste Strömungszelle eine bipolare Membran umfasst, die eine mit dem Katholyt in Kontakt stehende Kationenaustauschschicht und eine mit dem Anolyt in Kontakt stehende Anionenaustauschschicht enthält; wobei die Kationenaustauschschicht dem Katholyt Protonen zuführt und die Anionenaustauschschicht dem Anolyt Hydroxidionen zuführt; wobei der saure Katholyt einen pH-Wert von höchstens 5,5 aufweist und wobei der pH-Wert des Katholyten niedriger ist als der pH-Wert des Anolyten.

2. Das Verfahren nach Anspruch 1 ist **dadurch gekennzeichnet, dass** der aus dem Katholytbehälter austretende indirekte Gasstrom Kohlendioxid enthält und dass das Verfahren ferner einen Schritt e) umfasst, bei dem der aus dem Katholytbehälter austretende indirekte Gasstrom zurückgewonnen und in den Kohlendioxid enthaltenden Gaseinlassstrom aus Schritt d) zurückgeführt wird.

3. Das Verfahren nach Anspruch 1 oder 2 ist **dadurch gekennzeichnet, dass** der in Schritt (d) bereitgestellte Gaseinlassstrom eine Durchflussrate im Bereich von 0,5 bis 10 ml/min aufweist; vorzugsweise von 0,9 bis 2,8 ml/min oder von 1,0 bis 2,5 ml/min.

4. Das Verfahren nach einem der Ansprüche 1 bis 3 ist **dadurch gekennzeichnet, dass** der saure Katholyt einen pH-Wert im Bereich von 0,5 bis 5,4, vorzugsweise von 1,0 bis 4,0, aufweist.

5. Das Verfahren nach einem der Ansprüche 1 bis 4 ist **dadurch gekennzeichnet, dass** der Anolyt einen pH-Wert im Bereich von 7 bis 15, vorzugsweise von 10 bis 14, aufweist.

6. Das Verfahren nach einem der Ansprüche 1 bis 5 ist **dadurch gekennzeichnet, dass** der saure Katholyt eine oder mehrere Säuren in einer Konzentration im Bereich von 0,01 bis 1,0 M und einen oder mehrere Alkalimetallkationen-Donatoren in einer Konzentration im Bereich von 1,0 bis 5,0 M enthält.

7. Das Verfahren nach Anspruch 6 ist **dadurch gekennzeichnet, dass** das eine oder die mehreren Alkalimetallkationen eines oder mehrere sind, die aus Cs+, K+, Li+ und Na+ ausgewählt sind; vorzugsweise sind das eine oder die mehreren Alkalimetallkationen K+ oder umfassen K+.

8. Das Verfahren nach einem der Ansprüche 1 bis 7 ist **dadurch gekennzeichnet, dass** der saure Katholyt eine oder mehrere Alkalimetallkationen-Donatoren umfasst, ausgewählt aus Cäsiumchlorid, Cäsiumiodid, Cäsiumsulfat, Cäsiumphosphat, Cäsiumhydroxid, Kaliumchlorid, einbasischem Kaliumphosphat, Kaliumsulfat, Kaliumiodid, Kaliumhydroxid, Lithiumchlorid, Lithiumiodid, Lithiumsulfat, Lithiumphosphat, Lithiumhydroxid, Natriumchlorid, Natriumsulfat, Natriumiodid, Natriumphosphat und Natriumhydroxid; vorzugsweise ausgewählt aus Kaliumchlorid, einbasischem Kaliumphosphat, Kaliumsulfat, Kaliumiodid und Kaliumhydroxid; noch bevorzugter sind der eine oder die mehreren Alkalimetallkationen-Donatoren Kaliumchlorid oder umfassen Kaliumchlorid.

9. Das Verfahren nach Anspruch 8 ist **dadurch gekennzeichnet, dass** der eine oder die mehreren Alkalimetallkationen-Donatoren in einer Konzentration im Bereich von 0,5 bis 5,0 M, vorzugsweise im Bereich von 2,0 bis 4,0 M, vorliegen.

10. Das Verfahren nach einem der Ansprüche 1 bis 9 ist **dadurch gekennzeichnet, dass** der saure Katholyt eine oder mehrere Säuren umfasst, die aus Salzsäure, Schwefelsäure, Bromwasserstoffsäure, lodwasserstoffsäure, Perchlorsäure und Chlorsäure ausgewählt sind; vorzugsweise Schwefelsäure.

11. Das Verfahren nach Anspruch 10 ist **dadurch gekennzeichnet, dass** die eine oder mehreren Säuren in einer Konzentration im Bereich von 0,01 bis 1,0 M, vorzugsweise von 0,02 bis 0,5 M und noch bevorzugter im Bereich von 0,03 bis 0,2 M vorliegen.

12. Das Verfahren nach einem der Ansprüche 1 bis 11 ist **dadurch gekennzeichnet, dass** das Metall des metallbasierten Katalysators aus Kupfer, Silber und beliebigen Mischungen davon ausgewählt ist; und/oder der metallbasierte Katalysator aus Kupferoxid-Nanopartikeln besteht oder diese enthält und das Verfahren einen Katalysatoraktivierungsschritt umfasst, um Kupferoxid zu metallischem Kupfer zu reduzieren.

13. Das Verfahren nach einem der Ansprüche 1 bis 12 ist **dadurch gekennzeichnet, dass** die Betriebsbedingungen, unter denen die Durchflusszelle in Schritt c) betrieben wird, eine Stromdichte im Bereich von -100 mA/cm² bis -1,5 A/cm² umfassen; vorzugsweise im Bereich von -150 mA/cm² bis -800 mA/cm².

14. System (1), das zur Durchführung des Verfahrens zur Elektrolyse von Kohlendioxid gemäß einem der Ansprüche 1 bis 13 geeignet ist, wobei das System eine mit Gas gespeiste Durchflusszelle (3) umfasst, die eine Gaskammer (5), eine Katholytkammer (7) und eine Anolytkammer (9) umfasst, wobei die Gaskammer (5) von der Katholytkammer (7) durch eine Gasdiffusionselektrode (17) getrennt ist, wobei die Gasdiffusionselektrode (17) eine Gasdiffusionsmembran aufweist, die in der Gaskammer angeordnet ist, wobei die Katholytkammer (7) und die Anolytkammer (9) jeweils eine Kathode und eine Anode umfassen, und wobei das System (1) ferner Katholyt (23) und Anolyt (25) sowie Mittel (27; 29) zum Strömenlassen des Katholyten (23) und des Anolyten (25) jeweils innerhalb der Katholytkammer (7) und der Anolytkammer (9) umfasst;
wobei das System **dadurch gekennzeichnet ist, dass** der Katholytenstrom ein saurer Katholytenstrom ist, der ein oder mehrere Alkalimetallkationen enthält, und dass die mit Gas gespeiste Strömungszelle eine bipolare Membran (19) umfasst, die eine Kationenaustauschschicht in Kontakt mit dem Katholyt und eine Anionenaustauschschicht in Kontakt mit dem Anolyt enthält; wobei die Kationenaustauschschicht dem Katholyt Protonen zuführt und die Anionenaustauschschicht dem Anolyt Hydroxidionen zuführt; dass der saure Katholyt einen pH-Wert von höchstens 5,5 aufweist und dass der pH-Wert des Katholyten niedriger ist als der pH-Wert des Anolyten;
wobei das System (1) ferner einen Katholytbehälter zur Aufnahme und Entgasung des aus der Katholytkammer austretenden flüssigen Katholyt-Ausflusses umfasst, sowie vorzugsweise Mittel (31) zur Rückgewinnung eines aus dem Gasauslass (33) des Katholytbehälters austretenden indirekten Gasstroms und Mittel (35) zur Rückführung des genannten indirekten Gasstroms in die Gaskammer (5).

15. Verwendung eines Systems, das eine mit Gas gespeiste Durchflusszelle (3) mit einer bipolaren Membran (19) umfasst, in einem Verfahren zur Elektrolyse von Kohlendioxid unter sauren Bedingungen in Gegenwart eines oder mehrerer Alkalimetallkationen; wobei das System gemäß Anspruch 14 und/oder das Verfahren gemäß einem der Ansprüche 1 bis 13 ist.

## Revendications

1. Procédé d'électrolyse du dioxyde de carbone, ledit procédé étant **caractérisé en ce qu'**il comprend les étapes suivantes :
a) fournir un système comprenant une cellule d'écoulement alimentée en gaz comprenant une chambre à gaz avec une entrée de gaz, une sortie de gaz, une chambre de catholyte et une électrode de diffusion de gaz comprenant un catalyseur à base de métal, où l'électrode de diffusion de gaz est placée entre la chambre à gaz et la chambre de catholyte ;
b) fournir un flux de catholyte et un flux d'anolyte dans ladite cellule d'écoulement alimentée en gaz ;
c) activer ladite cellule d'écoulement alimentée en gaz dans des conditions de fonctionnement ;
d) fournir un flux d'entrée de gaz comprenant du dioxyde de carbone en utilisant l'entrée de gaz de la chambre à gaz pour produire un flux de gaz direct sortant de la sortie de gaz de la chambre à gaz et un flux de sortie de catholyte liquide provenant de la chambre de catholyte comprenant des produits, où ledit flux de sortie de catholyte liquide est dégazé dans un réservoir de catholyte pour produire un flux de gaz indirect sortant d'une sortie de gaz du réservoir de catholyte ;
où le flux de catholyte est un flux de catholyte acide comprenant un ou plusieurs cations de métaux alcalins et **en ce que** la cellule d'écoulement alimentée en gaz comprend une membrane bipolaire qui comprend une couche échangeuse de cations en contact avec le catholyte et une couche échangeuse d'anions en contact avec l'anolyte ; où la couche échangeuse de cations fournit des protons au catholyte et la couche échangeuse d'anions fournit des ions hydroxydes à l'anolyte ; **en ce que** le catholyte acide a un pH d'au plus 5,5 et **en ce que** le pH du catholyte est inférieur au pH de l'anolyte.

2. Le procédé selon la revendication 1 est **caractérisé en ce que** le flux de gaz indirect sortant du réservoir de catholyte comprend du dioxyde de carbone, et **en ce que** le procédé comprend en outre une étape e) de récupération du flux de gaz indirect sortant du réservoir de catholyte et de recyclage dudit flux de gaz indirect dans le flux d'entrée de gaz comprenant du dioxyde de carbone de l'étape d).

3. Le procédé selon la revendication 1 ou 2 est **caractérisé en ce que** le débit d'entrée de gaz fourni dans l'étape (d) a un débit allant de 0,5 à 10 ml/min ; de préférence de 0,9 à 2,8 ml/min ou de 1,0 à 2,5 ml/min.

4. Le procédé selon l'une quelconque des revendications 1 à 3 est **caractérisé en ce que** le catholyte acide a un pH allant de 0,5 à 5,4 ; de préférence de 1,0 à 4,0.

5. Le procédé selon l'une quelconque des revendications 1 à 4 est **caractérisé en ce que** l'anolyte a un pH allant de 7 à 15 ; de préférence de 10 à 14.

6. Le procédé selon l'une quelconque des revendications 1 à 5 est **caractérisé en ce que** le catholyte acide comprend un ou plusieurs acides à une concentration allant de 0,01 à 1,0 M et un ou plusieurs donneurs de cations de métaux alcalins à une concentration allant de 1,0 à 5,0 M.

7. Le procédé selon la revendication 6 est **caractérisé en ce que** le ou les cations de métaux alcalins sont un ou plusieurs cations choisis parmi Cs⁺, K⁺, Li⁺ et Na⁺ ; de préférence, le ou les cations de métaux alcalins sont ou comprennent K⁺.

8. Le procédé selon l'une quelconque des revendications 1 à 7 est **caractérisé en ce que** le catholyte acide comprend un ou plusieurs donneurs de cations de métaux alcalins choisis parmi le chlorure de césium, l'iodure de césium, le sulfate de césium, le phosphate de césium, l'hydroxyde de césium, le chlorure de potassium, le phosphate de potassium monobasique, le sulfate de potassium, l'iodure de potassium, l'hydroxyde de potassium, le chlorure de lithium, l'iodure de lithium, le sulfate de lithium, le phosphate de lithium, l'hydroxyde de lithium, le chlorure de sodium, le sulfate de sodium, l'iodure de sodium et l'hydroxyde de sodium ; de préférence choisis parmi le chlorure de potassium, le phosphate de potassium monobasique, le sulfate de potassium, l'iodure de potassium et l'hydroxyde de potassium ; le plus préférable étant que le ou les donneurs de cations de métaux alcalins soient ou comprennent du chlorure de potassium.

9. Le procédé selon la revendication 8 est **caractérisé en ce que** le ou les donneurs de cations de métaux alcalins sont présents à une concentration allant de 0,5 à 5,0 M ; de préférence allant de 2,0 à 4,0 M.

10. Le procédé selon l'une quelconque des revendications 1 à 9 est **caractérisé en ce que** le catholyte acide comprend un ou plusieurs acides choisis parmi l'acide chlorhydrique, l'acide sulfurique, l'acide bromhydrique, l'acide iodhydrique, l'acide perchlorique et l'acide chlorique ; de préférence l'acide sulfurique.

11. Le procédé selon la revendication 10 est **caractérisé en ce que** le ou les acides sont présents à une concentration allant de 0,01 à 1,0 M ; de préférence, de 0,02 à 0,5 M ; le plus préférable étant de 0,03 à 0,2 M.

12. Le procédé selon l'une quelconque des revendications 1 à 11 est **caractérisé en ce que** le métal du catalyseur à base de métal est choisi parmi le cuivre, l'argent et tout mélange de ceux-ci ; et/ou le catalyseur à base de métal est ou comprend des nanoparticules d'oxyde de cuivre et le procédé comprend une étape d'activation du catalyseur pour réduire l'oxyde de cuivre en cuivre métallique.

13. Le procédé selon l'une quelconque des revendications 1 à 12 est **caractérisé en ce que** les conditions de fonctionnement auxquelles la cellule d'écoulement est exploitée à l'étape c) comprennent une densité de courant allant de -100 mA.cm² à -1,5 A.cm² ; de préférence de -150 mA.cm² à -800 mA.cm².

14. Un système (1) approprié pour exécuter le procédé d'électrolyse du dioxyde de carbone selon l'une quelconque des revendications 1 à 13, le système comprenant une cellule d'écoulement alimentée en gaz (3) comprenant une chambre à gaz (5), une chambre de catholyte (7) et une chambre d'anolyte (9), où ladite chambre à gaz (5) est séparée de la chambre de catholyte (7) par une électrode de diffusion de gaz (17), ladite électrode de diffusion de gaz (17) ayant une membrane de diffusion de gaz étant comprise à l'intérieur de ladite chambre à gaz, où ladite chambre de catholyte (7) et ladite chambre d'anolyte (9) comprennent respectivement une cathode et une anode, et où le système (1) comprend en outre un catholyte (23) et un anolyte (25) et des moyens (27 ; 29) pour faire circuler le catholyte (23) et l'anolyte (25) à l'intérieur respectivement de ladite chambre de catholyte (7) et de ladite chambre d'anolyte (9) ; où le système est **caractérisé en ce que** le flux de catholyte est un flux de catholyte acide comprenant un ou plusieurs cations de métaux alcalins et **en ce que** la cellule d'écoulement alimentée en gaz comprend une membrane bipolaire (19) qui comprend une couche échangeuse de cations en contact avec le catholyte et une couche échangeuse d'anions en contact avec l'anolyte ; où la couche échangeuse de cations fournit des protons au catholyte et la couche échangeuse d'anions fournit des ions hydroxydes à l'anolyte ; **en ce que** le catholyte acide a un pH d'au plus 5,5 et **en ce que** le pH du catholyte est inférieur au pH de l'anolyte ;
et où le système (1) comprend en outre un réservoir de catholyte pour recevoir et dégazer le flux de sortie de catholyte liquide sortant de la chambre de catholyte , et de préférence, des moyens (31) pour récupérer un flux de gaz indirect sortant de la sortie de gaz (33) du réservoir de catholyte, et des moyens (35) pour recycler ledit flux de gaz indirect dans la chambre à gaz (5).

15. Utilisation d'un système comprenant une cellule d'écoulement alimentée en gaz (3) avec une membrane bipolaire (19) dans un procédé d'électrolyse du dioxyde de carbone dans des conditions acides en présence d'un ou plusieurs cations de métaux alcalins ; où le système est selon la revendication 14 et/ou le procédé est selon l'une quelconque des revendications 1 à 13.
